

Nov. 15, 1938.

M. O. SCHUR

2,136,826

MANUFACTURE OF MOLDED BINDER-REINFORCED  
FIBER ARTICLES OF PLIANT CHARACTER  
Filed Sept. 4, 1935

2 Sheets-Sheet 1



Nov. 15, 1938.

M. O. SCHUR

2,136,826

MANUFACTURE OF MOLDED BINDER-REINFORCED  
FIBER ARTICLES OF PLIANT CHARACTER

Filed Sept. 4, 1935

2 Sheets-Sheet 2



Inventor  
Milton O. Schur  
by Wright, Brem, Quincy, Day

Atty's.

Patented Nov. 15, 1938

2,136,826

# UNITED STATES PATENT OFFICE

2,136,826

## MANUFACTURE OF MOLDED BINDER-REINFORCED FIBER ARTICLES OF PLIANT CHARACTER

Milton O. Schur, Berlin, N. H., assignor to Brown Company, Berlin, N. H., a corporation of Maine

Application September 4, 1935, Serial No. 39,107

3 Claims. (Cl. 2—192)

This invention relates to the manufacture of molded, binder-reinforced, fiber articles of a pliant character, for instance, articles of a pliancy comparable to that of suede or of the felt in a true felt hat. It deals more especially with articles of the sort whose molded fibrous base is an interfelted, waterlaid one in the sense that it is deposited by flowing an aqueous fiber suspension onto a foraminous or wire mold through which the free water of the suspension drains or is sucked while the fibers are being matted or laid down in interfelted relationship as a layer conforming to the configuration of the mold.

In accordance with the present invention, various kinds of molded, binder-reinforced, fiber articles of a pliant character, for instance, hat shapes, are formed by depositing fibers of the appropriate character from aqueous suspension onto foraminous molds, the aqueous suspension carrying additionally, if desired, binder of suitable character so that the binder-reinforced articles may be formed in a single operation; or, if desired, the molded articles may be formed substantially without binder as sufficiently porous and absorptive structures to undergo readily a subsequent impregnating operation with suitable binder, the articles preferably being compacted and dried prior to such impregnation. While not limited thereto, the principles of the present invention are applicable to especial advantage in the fabrication of seamless hats whose appearance, feel, pliancy, toughness and other qualities are imitative of those of genuine felt hats. In such case, after the binder-reinforced hat shape has been produced as hereinbefore indicated, at least the external surface of the hat shape and preferably both its surfaces are finished with fiber flock to simulate in appearance and feel the surface of a genuine felt hat.

With the foregoing and other features and objects in view, I shall now describe my invention as applied to hat-making with particular reference to the accompanying drawings, wherein

Figure 1 is a section through one form of apparatus that may be employed for molding a hat shape, the apparatus including adjuncts for compacting and, if desired, drying the wet hat shape.

Figure 2 is a section through somewhat modified molding apparatus during the molding operation, with which apparatus a different type of instrumentality for compacting the wet hat shape is designed to be used.

Figure 3 is a similar view of the apparatus of Figure 2 after the molding operation and with the compacting instrumentality in place.

Figure 4 is a similar view of the same apparatus while compacting of the layer constituting the hat shape is being effected.

Figure 5 is a side view of the molded hat shape.

Before dealing with the particular fiber furnish, binders, and other materials employed in fabricating the hats of the present invention, it is perhaps well to describe the particular molding apparatus shown in the accompanying drawings, which apparatus, it is to be understood, is subject to considerable variation. The apparatus of Figure 1 comprises a cylindrical vat 10 into which an aqueous fiber suspension of the appropriate consistency, namely, of a fiber content usually not exceeding about 2%, is delivered from a suitable source of supply (not shown) by a valved pipe 11. In order to realize uniform interfelting of the fibers as they are being deposited from aqueous suspension, it is preferable to deliver very dilute fiber suspensions to the apparatus, for instance, suspensions of a fiber content of  $\frac{1}{2}$  to  $\frac{1}{4}\%$  or even lower. The apparatus as depicted in Figure 1 comprises only a single wire mold 12, but it is obvious that multiple-mold apparatus may be employed. The mold illustrated, which assumes the form of an inverted hat shape, may be constructed of wire cloth of a mesh and quality similar to that serving as the endless wire of a Fourdrinier papermaking machine or as the periphery of the cylinder mold of a so-called cylinder papermaking machine. Its marginal portion 13 may be fixed, as by welding, to the out-turned flanged upper end portion 14 of a cylindrical supporting frame 15 movable vertically out of the vat along with the mold carried thereby while guided in such movement by a cylindrical outer shell 16 with which it makes sliding contact. The lower end of the shell 16 may be fixed to the bottom 17 of the vat and its upper end may serve as the rest for the flanged upper end portion 14 of the frame 15. The pulp suspension delivered into the vat overflows an annular dam 18 arranged concentrically about the mold 12 and fills up the mold so as to deposit a substantially uniform layer of fibers 19 on the mold as the water of the suspension is draining through the mold into the compartment 20 defined by the shell 16. A valved pipe 21 for withdrawing the white water from the compartment 20 is kept open during the molding operation, which operation is preferably initiated with a supply of white water in the compartment 20 up to the very top of the mold, namely, to the level of its marginal portion 13, so as to avoid a "water-wing" effect, that is, an immediate sealing of the openings of the mold 55

by the water of the pulp suspension that prevents drainage of water therethrough. To this end, the valve 22 in the pipe 21 is preferably a two-way one designed to permit downward flow of white water from the compartment through its branch 23 during a molding operation and upward flow of white water through its branch 24 into the compartment before beginning a molding operation. Aqueous suspension of fiber in volume predetermined to deposit a layer of fibers 19 of the desired thickness on the mold is progressively delivered into the apparatus and the valved pipe 11 then closed.

Inasmuch as the hat shape 19 as deposited on the mold is too wet and pulpy to be removed from the mold or handled without damage, provision is made to compact and dewater it to a self-sustaining condition. To this end, the molding apparatus of Figure 1 includes means for raising the mold-supporting frame 15 while guided by the shell 16 out of the vat so as to bring the wet hat shape carried by the mold into pressing contact with a compacting instrumentality 25 of a configuration mating with that of the mold, as illustrated in dotted outline. Thus, the lower walls of the mold-supporting frame 15 may be bridged by a transverse bar 26 fixed in turn to the upper end portion of a plunger or reciprocatable rod 27 passing through a suitable stuffing box 28 into the compartment 20. Movement of the plunger may be effected by suitable means (not shown) to raise the wet hat shape carried by the mold 19 into pressing contact with the compacting instrumentality 25 and then to lower the mold to its molding position in the vat. If desired, the instrumentality 25, which may be constructed of suitable metal, such as steel, and be smoothly finished on its exterior, may have a hollow interior 29 into which steam or other suitable heating medium may be introduced by a pipe 30 so that upon bringing the wet hat shape into the desired pressing contact therewith, not only may the free water be squeezed from the shape but the shape may be partially or completely dried. Once the hat shape has been compacted and dewatered to a self-sustaining condition, so that it may be removed from the mold and handled without injury, a partial downward movement of the plunger 27 may be effected to permit the hat shape to be removed for further treatment, whereupon the remaining downward travel of the plunger may be completed.

The hat-molding apparatus shown in Figure 2 is essentially similar to that of Figure 1 excepting that no provision is made for raising the mold-support to bring the hat shape carried by the mold into pressing contact with a compacting instrumentality. On the contrary, the mold 40 appearing in the apparatus shown in Figure 2 is removably supported at its marginal portion 41 on an annular ledge 42 projecting inwardly from the upper portion of a cylindrical wall 43 upstanding from and fixed to the bottom of the vat and defining a compartment 44 into which white water drains from the mold during the delivery of aqueous fiber suspension thereon. Leading from the compartment 44 is a two-way valved pipe 21 having the same connections and the same functions as the similarly numbered pipe and connections of the apparatus of Figure 1.

The essential distinguishing feature between the apparatus of Figure 2 and that of Figure 1 is the means by which the wet hat shape 19 deposited on the mold is compacted and dewatered

to self-sustaining condition. Thus, as shown in Figure 3, after a wet hat shape has been deposited as previously described on the mold 40, a membrane 45 of rubber or equivalent stretchable and gas-impermeable material cemented or otherwise fixed to a rigid marginal retaining ring 46 is placed over the mold with the marginal portion of the membrane or the ring 46 making sealing contact with the marginal portion 41 of the mold. The membrane or diaphragm 45, which normally extends horizontally over the top of the mold so as to close off the top completely, is thus in a position to be sucked or stretched downwardly against the hat shape into the mold-conforming configuration shown in Figure 4, and, in so being stretched, to squeeze the free water from the wet hat shape and thus to compact it to a self-sustaining condition. The membrane may be placed under the appropriate suction by creating suction in the compartment 44 by opening a valved suction pipe 47 leading from such compartment to a vacuum chamber or pump (not shown). The valve 48 in the pipe 47 is preferably a two-way one, one way opening to a branch 49 communicating with the vacuum chamber or pump and the other to a branch 50 communicating with the atmosphere. After the desired compacting and dewatering of the hat shape has been accomplished, the suction branch 49 is closed and the atmospheric pressure branch 50 is opened to permit restoration of the compartment 44 to atmospheric pressure. In order to permit air to pass in between the membrane and the hat shape so as to break the suction that tends to persist therebetween and thus cause the membrane to peel away gradually from the hat shape and resume its normal unstretched position shown in Figure 3, the membrane is preferably provided, as at its center, with a valved, open-ended nipple 51 projecting upwardly therefrom, the membrane being cemented or otherwise sealed to a thin flange element 52 constituting the lower end of the nipple. The nipple is closed while suction is being applied to the membrane and is opened sufficiently when air is subsequently introduced into the compartment 44 to permit it to peel away gradually from the compacted and dewatered hat shape and thus to resume its normal unstretched position. The membrane and its rigid retaining ring 46 may then be removed from the mold, the mold and the hat shape carried thereby raised from its support, and the hat shape dried preferably while still carried by the mold, as in a hot air chamber.

Various binders may be used to impart the desired toughness and leather-like qualities to the fibrous body of the hat, for instance, such binders as rubber, glue, viscose, etc. These binders may be added to the aqueous suspension of fibers delivered to the hat-molding apparatus, in which case the white water system of the apparatus should preferably be maintained reasonably closed so as to utilize the binder carried away by the white water in preparing fresh or new fiber suspensions. In the case of rubber, the rubber may be added to the aqueous fiber suspension as at 4 to 6% fiber content in the form of rubber latex or artificial aqueous rubber dispersions and the rubber precipitated or coagulated on the fibers before being diluted with water for delivery to the molding apparatus; or a dilute aqueous suspension of flocculated or precipitated rubber may be separately prepared from rubber latex or other aqueous rubber dispersion

and admixed with the dilute aqueous fiber suspension immediately before its delivery to the molding apparatus. It may, however, be preferable to impregnate the premolded hat shape in 5 partially or completely dried condition. Thus, the premolded hat shape may be sprayed on either or both faces with rubber latex or other suitable binder to effect a substantial impregnation of its body; or, if desired, a substantially complete impregnation thereof.

Irrespective of whether the hat shape is molded in the presence of binder or whether binder is subsequently infused thereinto, it is then preferably surfaced with fiber flock so as to simulate 15 true felt or suede in its appearance and feel. If the hat is molded in the presence of binder and is then dried, it is necessary to apply suitable binder, such as rubber latex, glue, nitro-cellulose cement, etc., as by spraying, on the surface of the hat and then to shower fiber flock on the sticky hat surface as the hat is supported on a suitable form or block, with rotary or other appropriate movement of the form, if desired, to ensure substantially uniform flocking of the hat 20 surface with fiber. At least the outer surface of the hat is preferably thus finished with fiber flock; and it is usually desirable to turn the hat inside out on the supporting form after its outer surface has been finished and to finish the now- 25 outer surface in the same way as the previously outer surface. In those instances when the molded hat shape undergoes an after-impregnation with rubber latex or other suitable binder, as by spraying the binder on the shape while supported by a form or block, sufficient binder may be applied not only to effect impregnation of the body of the shape to the desired degree but to develop an adhesive coating on its surface which is showered with fiber flock and then permitted 30 to dry or set. Thereupon, if desired, the inside surface of the hat may be treated with binder and also flocked, as hereinbefore described. Of course, fiber flock of any suitable color or sheen may be employed; and, if desired, flock of one or 35 more colors may be distributed locally on the hat surface to produce highly ornamental effects, the binder for the flock and/or the flock being applied, for instance, through suitable stencils in producing such effects.

In some cases it is advantageous to form the hat into a shape which only roughly conforms to the final desired pattern, then re-wetting and stretching over a mold or form against which the material will shrink during re-drying. The hat 40 may then be flocked in the usual way. According to this procedure the number of relatively expensive foraminous molds necessary for the deposition of the pulp may be considerably reduced, and changes in final hat shapes may be effected 45 through the stretching process.

The flocked or finished hat may be given a final "blocking" or shaping as is customary in hat manufacture; and it may be provided with the usual accessory hat elements, such as a lining, 50 sweat band, etc., and the usual hat ornaments, such as an outer band or ribbon, buttons, feathers, buckles, etc.

An important factor in the realization of hats possessed of the desired body, feel, pliancy, and 55 other qualities is the character of the fiber furnish employed in molding the hat shape. Thus, unless the furnish is of the proper kind and is properly conditioned for the hat-molding operation, the resulting hat shape may be comparatively rigid or "boardy", as is true of the usual

molded pulp articles. In accordance with the present invention, I supply to the molding apparatus aqueous suspensions of cellulose fibers preferably in substantially unhydrated condition, for instance, suspensions of cellulose fibers of a difficultly hydratable character in such condition, typical of which fibers are wood pulps refined to high alpha cellulose content, say, an alpha cellulose content of about 92% to 98%, virgin cotton, mercerized wood pulps or cotton, and the like. 10 In suspending such fibers in water to form the dilute suspension delivered to the molding apparatus, care should be taken to avoid substantial beating or other intensive mechanical action such as is accompanied by a hydration or gelatinization of the fibers and consequent stiffness or boardiness in articles molded from the fiber suspensions. If desired, a portion of the fiber employed in the fiber suspensions delivered to the molding apparatus may be animal fibers, such as 15 wool and/or hair, in which case the cellulosic fiber portion of the furnish may be hydrated to a greater degree than is otherwise permissible, as 20 wool and/or hair are unhydratable and lend to the molded hat shape the desired pliancy and 25 other qualities. Indeed, when, say, 5% to 65% of wool and/or hair, based on the dry weight of the entire fibrous furnish constitutes, along with cellulose fiber, the fibrous furnish, it may be desirable to effect some degree of hydration or gelat- 30 inization of the cellulosic fibrous portion of the furnish in order to effect a binding or cementing together of the fibers of the hat base by the cellulose hydrate or gelatinized cellulose. Part of the fibrous furnish may be long-fibered pulps, such 35 as chemically pulped manila, sisal, ramie, etc., 5% to 50%, based on dry weight of the furnish, of such long-fibered pulp improving notably the results secured from furnishes containing a substantial proportion of mercerized cellulose fiber 40 and/or wool.

Various proportions of binder may serve as the reinforcing impregnant in the hat shape. Thus, the hat shape may contain from about 5 to 100% of rubber, or from about 8 to 40% of glue, or 45 from about  $\frac{1}{2}$  to 5% of cellulose regenerated from viscose, based on the dry weight of fiber in the hat shape. In the case of all of these binders and especially in the case of glue and viscose, it is desirable to introduce a suitable softening or 50 plasticizing agent into the hat shape in order to neutralize or offset such undesirable stiffening action of the shape as may come from the binder. Thus, hat shapes impregnated with dry rubber latex solids may to advantage contain about 5 to 55 25% of glycerine, based on latex solids; those impregnated with glue, about 75 to 200% of glycerine, based on glue solids; and those impregnated with about  $\frac{1}{2}$  to 5% cellulose regenerated from viscose, about 5 to 30% of glycerine, based on the 60 dry weight of fiber. Other softening agents, such as ethylene glycol or other homologues of glycerine, glucose or other invert sugars, "Nul-moline", and the like might be employed in lieu of glycerine. The glycerine or other softening 65 agent may be introduced directly into such impregnants as rubber latex, glue solution, and viscose, with which they are compatible; or they may be applied to the binder-impregnated hat shape either generally or locally, as in the form 70 of aqueous solutions. So, too, such stiffening agents as waterglass, starch paste, etc., may be added to the hat shape along with the binder. In some instances, binders such as rubber latex and glue, rubber latex and viscose, and rubber 75

5 latex, glue and viscose may be admixed to de-  
velop the proper degree of stiffness in the hat.  
In this connection, it might be noted that the  
addition of glue and/or viscose to a rubber latex  
binder has the effect of increasing the stiffness  
5 of the hat shape impregnated with the binder.  
As in the case of the softening agent, the stiff-  
fening agent may be infused into the binder-  
impregnated hat shape, as in the form of an  
aqueous solution; and such infusion may be had  
10 generally or locally, for instance, only at the brim  
portion of the hat, whereat greater stiffness is  
generally desired than at the crown portion.

15 While the thickness of the hat body or struc-  
ture prior to surfacing it with fiber flock is sub-  
ject to variation, it is generally the case that the  
thickness desired ranges from about 20 to 60 mils,  
as at such thickness it can be finished with fiber  
20 flock to produce a final hat structure or body  
whose thickness is comparable to that of suede  
or felt in a true felt hat.

I claim:—

25 1. A method of making a seamless, molded,  
binder-reinforced, waterlaid fiber article which  
comprises depositing fiber and an elastic binder  
from aqueous suspension into approximate arti-  
cle shape on a porous mold, compacting the arti-  
cle to remove free water therefrom and dewater-  
ing it to self-sustaining condition on said mold,  
30 removing the dried article from said mold, re-

wetting and stretching the article in rewetted  
condition to its final shape on another mold, and  
redrying the article on said other mold, thereby  
causing it to shrink against said other mold.

2. A method of making a seamless, molded, 5  
rubber-reinforced, waterlaid fiber article which  
comprises depositing fiber and flocculated rubber  
from aqueous suspension into approximate article  
shape on a porous mold, compacting the article  
10 to remove free water therefrom and dewatering  
it to self-sustaining condition on said mold, re-  
moving the dried article from said mold, rewet-  
ting and stretching the article in rewetted condi-  
tion to its final shape on another mold, and re-  
dry 15 ing the article on said other mold, thereby  
causing it to shrink against said other mold.

3. A method of making a seamless, molded,  
waterlaid fiber article which comprises deposit-  
ing fiber from aqueous suspension into approxi-  
mate article shape on a porous mold, compacting 20  
the article to remove free water therefrom and  
dewatering it to self-sustaining condition on said  
mold, removing the article from said mold,  
stretching the article, in whose body an elastic  
25 binder is incorporated as an impregnant, in the  
presence of moisture to its final shape on another  
mold, and drying the article on said other mold,  
thereby causing it to shrink against said other  
mold.

MILTON O. SCHUR. 30